

Feb. 1, 1944.

W. E. BEATTY

2,340,504

ABRASIVE

Filed March 1, 1943

*Fig. 1.*



*Fig. 2.*



*Fig. 3.*



INVENTOR.

BY

*W. E. Beatty*

ATTORNEY.

## UNITED STATES PATENT OFFICE

2,340,504

## ABRASIVE

William E. Beatty, Hollywood, Calif.

Application March 1, 1943, Serial No. 477,614

5 Claims. (Cl. 51—293)

The invention relates to an improvement in abrasives, such as carborundum wheels or saws, emery cloth or paper and the like.

Carborundum wheels about one-sixteenth of an inch thick and about nine or ten inches in diameter, are commonly used to cut steel rod or the like. Such wheels manufactured by the Carborundum Company and known as resinoid while commonly used to a large extent, have a serious drawback in that they are very fragile. For example, if such a wheel is held at one edge by the thumb and forefinger and it is tilted or swung slowly through the air, the chances are that the wheel will break. Many of them are broken in shipping and many others are broken in the course of trying to clamp them on the spindle. Also the periphery of such a wheel soon becomes jagged and as a jagged edge is liable to fracture the whole wheel when in use, it is common to discard such wheels after a short period of use and when they are still about eight inches in diameter.

It is assumed wheels of the particular type mentioned above comprise a plurality of different sizes of crystals of carborundum pressed in the shape of a wheel with a suitable binder. At any rate, the binder employed in such wheels as now available on the market results in a very brittle and fragile wheel, as pointed out above.

Aside from the above disadvantages in the use of such a wheel, a considerable amount of time is lost in the normal use of the wheel, for the reason that it is customary to try to avoid breaking the wheel when in use by bringing it lightly to the work then backing it off, waiting a while, then bringing it to the work again, commonly known as dancing the wheel on the work. Hence, the actual time that the wheel is in contact with the work forms only a small part of the total time consumed in cutting a steel rod.

An object of the present invention is particularly directed to increasing the strength of such wheels and this has led to the extension of the idea into analogous fields such as emery cloth or paper.

The following U. S. Patents 2,071,342, 2,133,076, 2,216,901 and 2,257,999 disclose the use of various coating compositions for the manufacture of translucent motion picture projection screens. Generally speaking, the coating composition may comprise cellulose acetate, or nitrate or ethyl cellulose, or benzyl cellulose, and a plasticizer, dissolved in a solvent. The above patents disclose various formulae which may be employed. The coating composition for screen manufacture,

is sprayed on a matrix which may be smooth or rough and the coating thus produced is stripped from the matrix and the resulting sheet is treated to render it translucent and suitable for the projection of the pictures.

According to the present invention, I make use of such a coating composition, although in its preferred form I add to it a suitable percent of resin as will be described later. This coating composition is applied to the carborundum wheels above described now on the market, by dipping, brushing or spraying, preferably the latter.

It has been discovered that such wheels are so porous that if the coating composition with sufficient thinner, is sprayed on one side of the wheel when it is supported flat, the coating composition will leak through the pores of the wheel, coat the channels through it as well as the opposite surface. The wheel thus coated may be air-dried or drying may be hastened by heating in an oven at about 250° F. for about ten minutes or more.

The result is that the coating composition forms a binder which interlocks all of the abrasive particles of the wheel together, and increases the strength and life of the wheel.

A preferred binder comprises ethyl cellulose in flake form, with a plasticizer such as triphenol-phosphate or the like, plus a resin such as taglac or beckacite, the latter being a phenolic resin, plus a solvent which may be one or more of the following: methyl alcohol, butyl alcohol, butyl acetate, and hydrocarbons such as toluol, benzol, and zylol.

While the above mentioned resin by itself is brittle, and no doubt this property is of advantage in holding the abrasive particles of the wheel together in their proper shape, by using from zero to 50% of the solids as one or more of the above resins, I still obtain a binder which is not brittle, but if it were applied to a flat matrix and stripped off as in screen manufacture, it would be found that the coating would be flexible and could be bent back and forth many times without cracking.

The characteristics of the preferred binder above mentioned are that it absorbs only a small amount of water, such as 2%, which is less than is true of some of the other cellulose compounds mentioned above. Also, a film of the preferred binder is very strong, as a film .001 of an inch thick will stand a pressure of about thirty pounds per square inch. The per cent of resin in the preferred binder could be increased to about 50%

of the solids and the resulting film would still be flexible. The resin increases the toughness of the film.

Another advantage of the preferred binder is that it retains its flexibility, strength and tenacity at temperatures as low as 70° C. below zero, and hence it does not become brittle in ordinary cold weather.

A carborundum wheel as above described, <sup>18</sup> of an inch thick, and known as resinoid, after having been discarded by a machine shop as being unfit for further use, although its periphery was not particularly jagged, was treated with the preferred binder above mentioned, using 10% resin, the binder solution was transparent, it was sprayed on one side of the wheel while it was supported in a horizontal position on a flat surface, the sprayed material seeped through the wheel to the underside thereof, and the wheel thus coated was put in an oven and baked at 250° F. for ten minutes. The wheel thus treated was stronger and more rigid than the untreated wheel. Its appearance to the eye of a casual observer was practically unchanged, because the coating composition is transparent and so near as can be determined a film approximately only .001 or .002 of an inch thick appeared on the opposite sides of the wheel, although it may have been much thicker than this in the interior pores of the wheel. The wheel felt slightly smoother to the touch and it still showed the usual rough surface on both sides thereof. It was heavier in weight showing that the binder had loaded the wheel. The wheel thus treated was tested by applying constant pressure to the wheel while it was employed to cut steel rod and it cut straight through without breaking, whereas this operation is not possible, or at least not practiced universally, with an untreated wheel. Also the wheel thus treated was able to cut straight through a drill about one-half inch in diameter by constantly keeping the wheel in contact with the drill, it not being necessary to repeatedly and lightly bring the wheel to the work as heretofore. Thus the work can be done in about one fourth of the usual time.

The coating and binding compositions as above described may also be used for other types of abrasives. It has been applied to the abrasive side of emery cloth. The coating composition seeped through the abrasive and coated the fabric beneath. The result was that some of the valleys in the abrasive side were filled up with the binder, the binder held the abrasive particles together and to the cloth, and the cloth thus coated was flexible and very much stronger and tougher than heretofore. The result of filling up some of the valleys in the abrasive is to prevent making deep scratches when using the cloth, whereby a more uniform polishing effect is obtained.

The binder composition above described may also be applied to sandpaper and to sand belts, by applying a coating thereof to the abrasive side, or to the backing side, or to both. This coating composition makes the backing more flexible and hence a sanding belt will conform more readily to the driving pulleys and reduce the slippage which is encountered with the comparatively stiff backings.

While the binder composition above described imparts considerable strength and body to the abrasive, whether in the form of a wheel or having a backing of cloth or paper or both or the like, this binder is very much softer than the

abrasive particles, and hence it readily wears away when the abrasive is moved across the surface of the work piece.

For further details of the invention reference may be made to the drawing wherein Fig. 1 is a plan view of a wheel coated according to the present invention.

Fig. 2 schematically illustrates a support for the wheel to be coated.

Fig. 3 is a greatly magnified sectional view on line 3-3 of Fig. 1, illustrating schematically the general arrangement of the coating composition as applied to a carborundum wheel one-sixteenth of an inch thick.

Referring to the drawing, the wheel 1 illustrates the carborundum wheel above described as now available on the market and having a central aperture 2, and the plastic coating or binder of this invention is indicated at 6.

In Fig. 2, 2 illustrates a base on which the wheel 1 may be supported when it is sprayed or brushed with the above described coating composition. The wheel 1 may be dipped in the composition if desired.

In Fig. 3, an attempt is made to schematically illustrate what apparently happens when the wheel is sprayed with the coating material, as found in the test above described. The carborundum crystals are indicated by the reference number 5. These crystals are at the present time apparently held together by a binder 9, which is supposed to be resin. In any event, it is very brittle with the defects above noted. The plastic coating and binding composition of this invention is illustrated by the portion 6 which is on one side of the wheel, this coating composition seeps through whatever channels it finds between the crystals 5, one such channel being represented at 7, and finds its way through the interstices of the crystals 5 to the opposite side where it forms the coating 8. If desired, however, the coating composition could be made a lot thicker so that it would not flow through so that it could be sprayed on opposite sides, but this is not necessary if sufficient solvent is employed to make it approximately of the consistency of rather thin sugar syrup. It will be apparent, therefore, that the abrasive particles 5 of the wheel 1 are interlocked with a plastic binder which has great strength even in thin films and which film taken by itself is flexible as distinguished from brittle.

If the coating solution is then enough, i. e. like thin sugar syrup, the channels such as 7 may in fact in the above test have been coated with a hollow tubular film of the plastic binder instead of solid threads as shown in Fig. 3, or both tubes and threads. In any event, after using the treated wheel above described for cutting a large number of steel pieces, the cutting edge of the wheel was examined and found to contain a large number of voids or hollows or depressions and its granular appearance was no different to the naked eye than an untreated wheel. The periphery was less jagged, if anything, than before. All the interstices between the grains 5 were not filled up with the film 6 which was very thin—a few thousandths of an inch thick—and this is desirable because it leaves depressions to reduce loading up as with untreated wheels, and facilitates the wheel to wear away when cutting soft metal such as dural, without burning the work. If desired however, multiple coats with drying or baking between each coat may be used until all the pores are filled and the abrasive particles are entirely encased in the plastic binder.

Also the use of the wheel in the above test did not result in any apparent stripping of the films 6 and 8 from the sides of the wheel, due no doubt to the interlocking of those films with the grains 5. The melting point of the material of films or coating 6 and 8, after the liquid coating has dried and solidified, is about 450° F. When the wheel 1 is cutting a work piece, if this temperature is approached, which seems unlikely, the coating 6 and 8 and in channels 7 would soften to facilitate breaking away the grains 5. At normal working temperatures, the binder of this invention has great strength, even in thin films. If desired, the coating composition can be applied only to the backing of paper or cloth for the abrasive particles. In fact it can be applied to the backing material per se, and the abrasive particles can be later applied and bound thereon with any suitable binder. Multiple coats can be used with drying or baking between successive coats. The backing thus produced is flexible, and very strong. Abrasive particles can be applied thereto in any suitable manner. As a later application of the liquid coating to a former dried film thereof will coalesce therewith due to the volatile solvent in the fresh liquid coating, a liquid coating of this material forms an excellent binder for abrasive particles to be cemented to a coated backing as above suggested.

Also the coating in liquid form may be applied, viz., sprayed on the underside of a fabric and as the coating impregnates the fabric and oozes to the top of the fabric, while it is still wet or tacky, and before it solidifies, abrasive particles may be sprinkled on the wet plastic on top of the fabric whereby the abrasive particles form facets in a solidified setting of the film or binder when it sets. Or, the liquid coating may be applied to the top of paper or fabric and the abrasive particles spread or sprinkled thereon before it sets. Multiple coats of the liquid binder and abrasive particles may thus be built up on the backing if desired.

One or multiple coats of the film 6 and 8 around the aperture 2 is desirable as such films not only strengthen the wheel but form in effect integral washers which are flexible and which further reduce the likelihood of the wheel 1 breaking when it is clamped on its driving spindle. If the coating solution is sprayed or applied to the top side of wheel 1 while resting on a flat support 4, the film on the underside of the wheel will have a flat surface, the replica of the support, if an excess of the coating solution is used. This is de-

sirable adjacent the aperture 2 and can be used throughout the whole of the side of the wheel, but has not been found necessary.

To prevent the solution from adhering to support 4, it should be noncompatible with the solution and may be of the nature set forth in the above patents or others of the same patentees, although other materials may be used.

As the dried films 6 and 8 are very thin and transparent, the marking and label on the untreated wheel are just as visible after the wheel has been treated. However, to distinguish a treated from an untreated wheel, the coating solution may have a suitable dye or color added to it.

I claim:

1. The process which comprises interlocking abrasive particles by applying thereto a solution of ethyl cellulose.
2. The process which comprises interlocking abrasive particles by applying thereto a solution of ethyl cellulose, a plasticizer and resin, the amount of resin being less than about 50% and insufficient to form a brittle film.
3. In an abrasive device having abrasive particles held by a binder, the improvement which comprises a coating of plastic flexible film forming material on said particles and binder, said coating comprising ethyl cellulose, synthetic resin and a plasticizer.
4. The process of adding a secondary binder to a preformed porous abrasive article having abrasive particles secured by a primary binder, said process comprising supporting the abrasive article in a horizontal position on a matrix and applying a liquid solidifiable binder to the article, said binder comprising a solution of ethyl cellulose, a plasticizer and synthetic resin the binder being thin enough to seep through the pores of the article and flow on the matrix, allowing the article thus coated to set, and stripping the same from said matrix.
5. The process of reinforcing a thin porous abrasive disc which comprises supporting said disc in a horizontal position on a matrix, and applying on said disc a liquid binder comprising a solution of ethyl cellulose, a plasticizer and synthetic resin, said solution being thin enough to impregnate said disc and seep through the pores of said disc and flow on the matrix under said disc, allowing the coating thus formed on the disc to set and stripping the coated disc from said matrix.

WILLIAM E. BEATTY.